

United States Patent [19]  
Peisach

[11] 3,910,793

[45] Oct. 7, 1975

[54] **RADIOGRAPHIC DIFFUSION TRANSFER ELEMENT**

2,861,885 11/1958 Land..... 96/29  
3,433,950 3/1969 Erikson..... 96/29

[75] Inventor: **Joel M. Peisach**, Hudson, Mass.

FOREIGN PATENTS OR APPLICATIONS  
901,163 6/1962 United Kingdom..... 96/82

[73] Assignee: **Polaroid Corporation**, Cambridge, Mass.

Primary Examiner—Norman G. Torchin

[22] Filed: **Oct. 5, 1970**

Assistant Examiner—John L. Goodrow

[21] Appl. No.: **78,229**

Attorney, Agent, or Firm—John P. Morley

**Related U.S. Application Data**

[57] **ABSTRACT**

[63] Continuation of Ser. No. 655,197, July 21, 1967, abandoned.

A diffusion transfer photographic product useful for obtaining positive X-ray images and reradiation concentration measurements. Essentially, the product comprises a plurality of layers which include an intensifier-emulsion layer superposed above a reflecting layer integrated with a diffusion transfer capability for producing positive image patterns from the exposed intensifier-emulsion layer.

[52] **U.S. Cl.**..... 96/76 R; 96/82

**11 Claims, 4 Drawing Figures**

[51] **Int. Cl.**..... G03C 1/48

[58] **Field of Search**..... 96/82, 29, 76

[56] **Reference: Cited**

**UNITED STATES PATENTS**

1,315,324 9/1919 Mutscheller ..... 96/82





FIG. 1



FIG. 2



FIG. 3



FIG. 4

## RADIOGRAPHIC DIFFUSION TRANSFER ELEMENT

This is a continuation of application Ser. No. 655,197, filed July 21, 1967 and now abandoned.

This application relates to photography and more particularly to novel radiographic products and processes.

It is an object of this invention to provide novel products and processes particularly useful in X-ray photography, as well as for radiation detection means.

Another object is to provide improved products and processes for obtaining positive X-ray images and radiation concentration measurements by diffusion transfer techniques.

A principal object of this invention is to provide novel photosensitive elements wherein a silver halide emulsion and an X-ray intensifier screen are combined into a single layer, and this single layer is used in conjunction with a reflecting layer.

Other objects of the invention will in part be obvious and will in part appear hereinafter.

For a fuller understanding of the nature and objects of the invention, reference should be had to the following detailed description taken in connection with the accompanying drawing wherein:

FIG. 1 illustrates in diagrammatic enlarged cross-sectional view, an embodiment of this invention wherein a support 15 bears on its surface a reflectant dispersed in a suitable matrix 14, which in turn bears on its surface a layer 13 of a silver halide emulsion containing particles of a luminophor dispersed therein. This layer 13 is overcoated with an opaquing layer which optionally may serve as an antiabrasion coating;

FIG. 2 is a diagrammatic enlarged cross-sectional view showing the novel product of this invention adapted for use in diffusion transfer photography, prior to the application of the processing composition, the thickness of the various materials being greatly exaggerated for purposes of illustration;

FIG. 3 illustrates another embodiment of the invention adapted for use in diffusion transfer photography wherein the image-receiving layer 12 is loosely bonded to the photosensitive layer 13, and said layers are separated from each other by spreading of the processing composition contained in pod 16; and

FIG. 4 illustrates a badge, wall plaque or other suitable container designed to hold a photosensitive product within this invention prior to processing when the product is used as a radiation detection means.

It is known to prepare radiographs by diffusion transfer processes. U.S. Pat. No. 2,565,378, issued to Edwin H. Land on Aug. 21, 1951, discloses such a diffusion transfer process for preparing X-ray images, as does U.S. Pat. No. 3,185,841, also issued to Edwin H. Land, on May 25, 1965. U.S. Pat. No. 2,887,379, issued to Blake et al on May 19, 1959, discloses a film structure containing an intensifier screen, which may be utilized in diffusion transfer processes for obtaining X-ray images.

The use of intensifier screens in radiography is well-known. As is understood in the art, such screens are employed primarily to reduce the amount of exposure to X-ray or other radioactive waves necessary to form a latent image. Use of such screens also gives a more desirable, i.e., longer, contrast range curve. The advantages to be obtained by subjecting living organisms to lesser amounts of radiation are well-known to those fa-

miliar with the radiographic art. Accordingly, it has become quite common to employ such screens in radiography.

The generic term luminophor is subclassified into two categories; namely, fluorophors, i.e., fluorescent materials, and phosphors, i.e., phosphorescent materials. A luminophor has the property of being able to convert a part of the energy absorbed from activation by exposure to particular wavelengths of the spectrum, e.g., X-rays, into emitted radiation of a lower energy than the absorbed radiation, e.g., visible light, the lower energy radiation being in excess of associated thermal radiation. Fluorescent materials continue to emit radiation essentially only during the period of excitation.

There is a minimal afterglow. Phosphorescent materials, on the other hand, will continue to emit energy upon the cessation of the excitation of the luminophor. A phosphorescent material is said to possess an afterglow, i.e., continuance of emission after cessation of excitation, longer than about  $10^{-8}$  seconds for optical photons, whereas for fluorescent materials the afterglow is less than  $10^{-8}$  seconds. The basis for the demarcation at  $10^{-8}$  seconds between fluorescence and phosphorescence is explained in detail in *An Introduction to Luminescence of Solids* by Humboldt W. Leverenz, published by John Wiley and Sons, Inc., 1950, at page 149, et seq.

In general operation, a penetrable ionizing radiation package is exposed to, for example, X-ray radiation. The silver halide stratum possesses low stopping power for X-ray radiation. Thus, it permits the radiation to penetrate through it to the luminophor of the intensifier screen. The luminophor, upon absorbing X-ray radiation, will emit quanta in a particular segment of the electromagnetic spectrum. The photosensitive stratum is then exposed by the quanta emitted from the luminophor. Usually these quanta are in the form of visible light. The amount of quanta received by the photosensitive element is proportional to the degree of X-ray excitation of the luminophor at a given level of X-ray tube voltage. Thus, it is seen that latent image formation is derived from bombardment with two sources of quanta; namely, directly by the X-rays, and indirectly from the visible light emitted by the luminophor. It therefore follows that the use of an intensifier screen results in a lowering of the exposure dosage and/or the amount of radiation necessary to form the latent image.

The radiographic element of the present invention comprises the use of a dual function intensifier-silver halide emulsion layer used in conjunction with a superposed reflecting layer. The dual function layer can be prepared by admixing particles of a luminophor which is activatable substantially only by invisible radiation directly into the photosensitive silver halide emulsion material and laying this combination down as one layer, preferably upon a reflecting layer.

The combined intensifier-emulsion of the present invention utilizes the same principles to obtain exposure of the silver halide present as in the prior art X-ray packages previously discussed. Whereas the prior art utilized a physically distinct separate, intensifier layer (coated in intimate contact with the emulsion or else a separate intensifier screen that is placed in a superposed coextensive planar relationship with the emulsion), the present invention uses but a single layer that contains particles of luminophor as well as particles of silver halide within the binding agent. Here the quanta

of X-ray radiation penetrate into the binding agent, strike the particles of luminophor which are in turn excited and are thus induced to emit light, primarily in the visible part of the spectrum, to expose the grains of silver halide present.

The advantages to be gained from a utilization of an integral system of the present configuration are several fold. In the first instance, only one coating operation is involved as opposed to the multiplicity of coatings in previous integral systems.

The close proximity of the luminophor particles to particles of emulsion gives rise to a more efficient utilization of the excited luminophoric material. It is seen therefore that the flow of visible light emitted from each particle of luminophor has less chance of being impeded by another particle of luminophor prior to striking a silver halide grain. This better utilization of the luminophor gives rise to an increase in "package efficiency" over the conventional separate screen and separate silver halide emulsion.

Package efficiency as used herein is the total efficiency of all of the components of a photographic system in its ability to translate high energy invisible radiation into a high quality, high contrast photographic image. It is the sum of the inherent photosensitivity of the negative, the efficiency of the diffusion transfer processing composition in its ability to amplify a latent image, the ability of the luminophor to convert essentially invisible ionizing radiation to visible light, and the ability of receiving material to deposit positive silver in such a manner that maximum covering power is obtained.

It was also found that as a result of this close proximity of the luminophor to the silver halide that diffusion transfer images of a higher resolution were obtained than were obtained from the diffusion transfer separate intensifier screen system utilizing similar kilovolt dosages of X-ray radiation and similar amounts of phosphor per unit area.

The reflecting layer provides a more efficient utilization of the light emitted by the luminophoric particles. As is known, when the luminophoric particles are activated by penetrating ionizing radiation, the light quanta emitted travel omnidirectionally. It has been found that about 54 percent of this emitted light quanta is transmitted out of the intensifieremulsion layer. It has been found that by using a "back-scattering" or reflecting layer, an increased efficiency of 30-50 percent is obtained in the use of this emitted light as a result of its reflection back into the photosensitive layer. This efficiency increase is obtained without an appreciable loss in resolution.

It will be appreciated that the incorporation of the luminophor into the photosensitive emulsion actually amounts to a pigmentation of the emulsion. It was found, however, that one could still obtain high quality diffusion transfer reflection prints, with little or no loss in resolution, using such dual function silver halide layers.

It has previously been proposed, in British Pat. No. 901,162, to incorporate small quantities of a luminophor into a conventional wet developed silver halide emulsion. Only exceedingly small ratios of luminophor to silver, no greater than 5:1 or 6:1 may be employed since negatives which contain higher amounts of luminophor will not readily transmit light. A conventional negative that contains between 1,500 and 2,000

mg/sq. foot of silver and utilizes a 20:1 ratio of luminophor to binder would contain 3 to 5 grams of luminophor per square foot. When this amount of luminophor was coated upon a transparent support for the purposes of conducting a light transmission test, it was found that only about 25-40 percent of the incident light striking the test panel was transmitted. The amount transmitted by a silver halide emulsion containing this amount of luminophor would be approximately 50 percent less. (Measurements were made on a transmission densitometer having a 30 watt tungsten source, manufactured by the Muehle Corp., Newburgh, N.Y.) Satisfactory prints could not be obtained from such a negative as a practical matter because of this exceedingly low light transmission.

In contradistinction to a wet developed negative of the type just discussed, diffusion transfer radiographic images are formed in a different layer and their optical properties are essentially independent of the quantity of luminophor in the silver halide emulsion. The amount of luminophor that can be added to the silver halide emulsion in accordance with this invention is governed by the physical volume available for "packing" luminophor into the binder. This amount is independent of the translucency factor but is, of course, dependent upon the mean particle size of the luminophor. In addition, the photosensitive elements of this invention may, and preferably do, contain a reflecting layer as discussed above. Such reflecting layers could not be used in the negative materials of the aforementioned British patent, and their benefits thus were unavailable to one practicing that disclosure.

The utilization of such luminophor-silver halide layer in accordance with the present invention may best be understood by referring to the drawing.

FIG. 1 illustrates one embodiment of this invention wherein the several layers are coated upon each other. FIG. 2 illustrates an embodiment of the invention specifically adapted for diffusion transfer processing employing the element of FIG. 1. A rupturable container of processing solution, such as that disclosed in U.S. Pat. No. 2,565,378, is provided between the intensifieremulsion layer 13 and the receiving layer 12. A suitable support 15, such as those of a nature to be described below, is provided for both the receiving layer 12 and the intensifier screen-photosensitive emulsion 13, i.e., the layer containing the luminophor as well as the silver halide. The radiographic product illustrated in FIG. 2 is meant to be utilized in a diffusion transfer process similar to those previously described. Subsequent to exposure, the rupturable container 16 is broken, for instance, by passage between a pair of rollers, and the processing composition spread in a uniform layer between the emulsion layer containing the latent image and the receiving layer.

At some time subsequent to exposure, luminophoremulsion layer 13 containing the latent image is contacted with a processing composition preferably applied as a relatively viscous layer by rupture of pod 16. The processing composition may be any of those known in the art, e.g., a film-forming processing composition such as those disclosed in U.S. Pat. Nos. 2,543,181 and 2,565,378. It may comprise, for example, a developing agent such as hydroquinone, an alkali such as sodium hydroxide, a silver halide complexing agent such as sodium thiosulfate, and a high molecular weight film-forming thickening agent such as hydroxy-

ethyl cellulose or sodium carboxymethyl cellulose. Various other additives such as accelerating developing agents, preservatives, antifogging agents, and the like may also be included. All of these materials are preferably in aqueous solution. These photographic agents are preferably contained in solution in the processing liquid prior to the spreading thereof, but one or more of them may be in part or wholly located in the film element and dissolved into the applied processing composition.

When the embodiment set forth in FIG. 2 is processed through a pair of rollers or other spread system in conformance with the well-known diffusion transfer processing techniques, the ingredients of the processing composition help to maintain an intimate contact between the receiving material and the photosensitive element during imbibition. After processing, the image-receiving material is stripped from the integral emulsion-intensifier screen unit and the latter is discarded.

It is also within the scope of this invention to coat the image-receiving layer over the dual function intensifier-emulsion layer, and to maintain said layers as an integral unit after processing. The luminophor effectively masks the developed silver in that layer. In addition, the luminophor remains activatable by ultraviolet light; placing the integral unit in a source of ultraviolet light will result in increased light being reflected through the silver transfer image to the observer, thereby increasing the effective contrast scale of the image.

FIG. 3 illustrates yet another embodiment of the invention utilizing a "preformed laminate" film format of the type shown in FIG. 10 of U.S. Pat. NO. 3,053,659. In this embodiment, the element containing the image-receiving layer 12 is bound in place to the element containing the luminophor-emulsion layer 13, a stripping layer 17 being positioned between said layers. The stripping layer is permeable by the processing composition and facilitates separation of the emulsion layer from the image-receiving layer in such a manner that the plastic film obtained from the film-forming material of the processing composition will preferentially adhere to the photosensitive layer 13. A suitable reagent for such a stripping layer is cellulose acetate hydrogen phthalate. It should also be noted that the rupturable container or pod 16 that holds the processing composition is positioned so as to discharge its contents between the stripping layer and the luminophor-emulsion layer.

It will be recognized that the novel photosensitive elements of this invention may be utilized to advantage, by virtue of their increased efficiency to record incident invisible radiation, to detect other invisible radiation besides X-ray, e.g., alpha, beta, and low level gamma particles. The system of this invention allows for a highly sensitive autoradiographic image recording medium. Typical areas where such monitoring is necessary include dentists' offices, research laboratories, atomic power plants, etc. and anywhere else that humans and animals might be exposed to sources of penetrating ionizing radiation.

Film badges as such for radiation detection, i.e., dosimeters, are not new in the art. Examples of film badges can be found, for example, in U.S. Pat. Nos. 2,483,991 and 2,659,013. However, the badge embodiment of the present invention comprises the first such badge wherein a luminophor is found in the same layer as the silver halide, and the first such badge wherein the

photosensitive element can comprise if desired, a single layer film which contains both a luminophor and the silver halide. Optionally, one may incorporate the desired opacifying and reflecting layers into the film badge holder instead of placing such layers in the photosensitive element itself. It will be appreciated, however, that the reflecting layer will be less effective if incorporated into the holder instead of being part of the photosensitive element.

10 FIG. 4 is a perspective view of a badge or wall plaque adapted to hold a photosensitive element such as the embodiment of FIG. 1 when such is to be used as a radiation detection system. The badge comprises any suitable holder 20 having a retaining means for a radiosensitive element, an inlet portion 22 for the insertion and removal of said element, and means (not shown in this view) for adhering the holder to an article of clothing, or to a solid surface such as a wall, a portion of said badge opposite said element 21 being capable of penetration by ionizing radiation. The holder may be of any known plastic or metal known in the art as useful for such purposes, and the portion penetrable by ionizing radiation may be merely an aperture in the holder or a substance such as polyethylene. Upon removal from the holder, the exposed photosensitive element may be processed in the same manner as the embodiment of FIG. 2.

Support 15 is either opaque to visible radiation and 30 transparent to X-rays and other radioactive rays, or, comprises a transparent base material, preferably a plastic, for example, a cellulosic ester such as cellulose acetate, or a synthetic polymer such as polyvinyl chloride, polyvinyl acetate, polystyrene, and polyethylene terephthalate, etc. Where the support is transparent, it will be apparent that it must be provided with a light-opaque backing, such as a black dye dispersed in a suitable medium, (e.g., gelatin) as is known in the art, or the film unit must otherwise be encased in a light-25 opaque material to prevent exposure to visible light.

Reflecting layer 14 may comprise a suitable reflecting agent such as barium sulphate, magnesium sulphate, titanium dioxide or zinc oxide dispersed in a suitable medium such as gelatin, polyvinyl alcohol or 45 polyethylene. The concentration of reflectant within the binder can vary such that the layer when considered as a separate entity can be translucent or opaque to visible light. Means for preparing such reflecting layers are well-known in the art; note, for example, the 50 aforementioned U.S. Pat. No. 3,053,659. In a preferred embodiment, this layer contains sufficient reflectant so as to act as an opaquing layer for the juxtaposed intensifier-emulsion layer.

The luminophors used in the intensifier-emulsion 55 layer may comprise any phosphorescent or luminescent luminophor known in the art, which is susceptible to excitation substantially only from penetrating ionizing radiation, e.g., X-ray radiation. Particularly satisfactory results may be obtained utilizing the following phosphorescent materials as the luminophor:

1. ZnS : Ag
2. ZnMgF<sub>2</sub> : Mn
3. ZnCdS : Cu
4. ZnO : Zn
5. MgF<sub>2</sub> : Mn
6. ZnS : Cu
7. ZnCdS : Ag

Particularly satisfactory results may also be obtained utilizing the following luminescent materials as the luminophor:

1. ZnS : Ag
2. ZnS : O<sub>4</sub> : Mg
3. ZnO : Zn
4. ZnS : Cu
5. ZnCdS : Ag
6. CdS : Ag
7. CaZnPO<sub>4</sub>
8. CdBO<sub>4</sub>
9. MgWO<sub>4</sub>
10. BaTiPO<sub>4</sub>
11. CaSiO<sub>4</sub> : Mg
12. Y<sub>2</sub>O<sub>3</sub> : Eu
13. YVO<sub>4</sub> : Eu
14. ZnSiO<sub>4</sub> : Mn
15. KMgF<sub>3</sub> : Mn
16. ZnSe : Cu
17. CaWO<sub>4</sub>
18. ZnS : Mn
19. LaBaO<sub>4</sub>
20. CaMgSiO<sub>3</sub> : Ce

Members of this class of luminophors emit light in the range from 375 to 620 millimicrons, or essentially, throughout the whole visible spectrum, and are activated only by radiation within the range of about 200 to about 360 millimicrons.

It has been found that satisfactory radiographic images can be obtained by use of a luminophor to silver ratio of 1:1 to 20:1 and a gelatin to silver ratio of 2:1 to 15:1. This intensifier-emulsion is coated upon the support with a luminophor coverage of about 0.1 to about 2.0 mg. per square centimeter within an emulsion of 100 mg. per square foot of silver halide coverage. Particularly beneficial results may be obtained by use of luminophor mean particle sizes of 3 to 12 microns and luminophor to silver ratios of about 7:1 to about 20:1.

The radiographic elements of the present invention may contain sufficient luminophor in the emulsion to "opaque" the emulsion. That is, the concentration of luminophor can prevent white light striking the surface of the intensifier-emulsion layer from exposing silver halide grains within the layer. However, since the luminophor can be activated by ultraviolet light which is to be found in sunlight as well as incandescent and fluorescent light sources, exposure to such ultraviolet light will cause the luminophor to emit radiation which will fog the grains. The use of an opacifying layer 11 which is penetrable only by ionizing radiation is recommended for placement on the exposed surface to prevent such undesired indirect fogging. This opaquing layer will also prevent direct fogging by white light sources of those grains which by a statistical basis happen to be on the surface of the layer. Such an opacifying layer may comprise, for example, carbon black or a black dye in a suitable matrix, such as gelatin. The opacifying layer must be permeable to the alkaline processing composition so that it will not interfere with the formation of the desired silver transfer image. The opacifying layer may also be utilized as an antiabrasion layer, as is conventional with anti-halation layers.

In the X-ray systems of the present invention, it is not necessary to quench the phosphor prior to developing the image. The failure to quench a phosphorescent luminophor when such is used in a non-integral X-ray

package would result in exposure in the previously unexposed areas should one attempt to move the film while phosphorescence is still occurring. In the present invention, there is a continuous point-to-point relationship between the silver halide and the luminophor due to the dual function of the single layer. This positioning of the intensifier material in relation to the silver halide is such that the problem of ghost images which could arise from the utilization of a phosphorescent intensifier cannot arise in the process of the present invention. Thus it is seen that movement of the intensifier, since it is in fixed relationship to the silver halide, i.e., it is all in one layer, will have no detrimental effect upon the latent image.

15 If a phosphorescent luminophor is utilized, it should be noted that said phosphorescent luminophor is not quenched by the processing composition but rather the silver halide solvent of the diffusion transfer processing composition complexes the unexposed silver halide and starts the imbibition process. The developing agent in the processing composition reduces the exposed silver halide to silver. The silver halide which was not exposed, by the incident radiation and/or the radiation emitted from the luminophor, is complexed and transferred to the receiving layer. Thus, while the luminophor particles may continue to phosphoresce, the effect is nullified such that the effect is the same as if quenching had taken place, whereas with a luminescent luminophor, when such is used, the quenching need never arises since excitation ceases at the cessation of radiation exposure.

The image-receiving layer 12 may be any of those useful in photographic diffusion transfer processes. In a preferred embodiment, image-receiving layer 12 comprises an image-receiving layer containing deacetylated chitin, which is described and claimed in the U.S. Pat. No. 3,087,815, issued to Ryan et al.

The emulsion material may be any suitable photosensitive silver halide emulsion known in the art. Particularly satisfactory results were obtained when a standard silver bromide emulsion that contained up to 10 mol percent of silver iodide was used. Conventional silver halide binders such as gelatin had no adverse effect upon the activity of the luminophor and in turn the luminophor brought about no detrimental effects such as de-sensitization of the silver halide. It was further determined that there was substantially no chemical interaction between the silver halide and the luminophor.

50 When the embodiments of the invention are utilized for diagnostic radiographic imaging, the use of higher X-ray voltages is facilitated since the actual exposure time may be of a shorter duration than that commonly required with the use of a separate screen and separate emulsion of a non-integral system.

55 Satisfactory results have been obtained utilizing a kilovolt range of 40 to 130 kv., the choice being dependent upon the ability of a particular luminophor to absorb the ionizing radiation as well as on the nature of the subject.

60 The use of the higher voltages insures minimal absorption of ionizing radiation by the subject. This is true because the higher the voltage the less the absorption, due to the greater proportion of "hard" X-rays which are the deep penetrating short wave length X-rays. These rays are least absorbed by the human body. The danger that arises from the soft X-rays is the fact that upon absorption by the body, they give rise to an

ionizing effect upon certain constituents of the body chemistry.

The following examples are intended to show by illustration only, and not in a limiting sense, the preparation of photosensitive elements and their use in accordance with this invention.

#### EXAMPLE I

22 cc. of 10 percent gelatin were mixed with 5 cc. of a standard silver halide emulsion and with 1.1 cc. of Triton X-100, a non-ionic isoctylphenylpolyethoxyethanol dispersing agent, trade name of and marketed by Rohm and Haas Company, Philadelphia, Pa. 10 grams of luminescent zinc sulfide were added and stirred for several seconds to insure a uniform mixture. This still liquid mixture was put into a syringe and sprayed onto a suitable support, and stroked with a "Myrod" — a steel wire bound rod — to insure a smooth layer. The cast layer was allowed to air dry.

#### EXAMPLE II

A base comprising paper overcoated with  $TiO_2$  dispersed in polyethylene was coated with a layer of luminescent zinc sulfide, activated with copper, dispersed in an X-ray type emulsion containing 97 percent silver bromide and 3 percent iodide. The coating was of a coverage of 1.7 grams of luminophor per square foot of base, and the silver concentration was 100 mg. per square foot of base. The gelatin to silver ratio was 4:1. An emulsion containing particles of intensifier screen material was thereby formed on the reflecting base after drying. A black dye in a gelatin matrix as an opaques and anti-abrasion layer was then overcoated onto the emulsion-intensifier layer.

#### EXAMPLE III

A sheet of the photographic film prepared as in Example 2 was given a 30 second unscreened X-ray exposure at 68 k.v.p., 100 MA. 40-inch distance through an aluminum step wedge. A positive transfer image was then obtained, in accordance with conventional diffusion transfer techniques, by imbibing the X-ray exposed film for 30 seconds through the permeable black dye layer with a developing composition similar to the one used in Polaroid Type 47 Land film. The positive image was revealed by stripping the silver receiving layer from the silver halide emulsion layer.

#### EXAMPLE IV

A conventional system employing a separate intensifier screen and separate superposed emulsion, wherein the intensifier screen comprises the same luminophor with the same coverage per unit area, was similarly exposed to X-ray radiation of the same kilovoltage. Time duration, distance, etc. were held constant. A control system comprising emulsion only without the presence of any luminophoric material was exposed in the same manner. Both of these radiographically exposed elements were processed in the same manner as was the sheet prepared in Example 1. Both samples that utilized a luminophor displayed a greater efficiency as to the utilization of invisible radiation to form a visible image. The system of the present invention required 25 percent of the radiation required by the control system to obtain similar images. The material of Example 1 required 50 percent less radiation than the conventional

separate screen-separate emulsion system to obtain the same sensitometric results.

For convenience, the expression "X-ray" has been used in the specification and in the claims and is intended to cover all photographically useful radioactive rays such as those emanating from an X-ray tube, radium, or radioactive isotopes.

Since certain changes may be made in the above product and process without departing from the scope of the invention herein involved, it is intended that all matter contained in the above description or shown in the accompanying drawing shall be interpreted as illustrative and not in a limiting sense. The invention accordingly comprises the products possessing the features, properties and relation of components, and the processes involving the several steps and the relation and order of one or more of such steps with respect to each of the others which are exemplified in the foregoing detailed disclosure, and the scope of the application of which will be indicated in the claims.

I claim:

1. An integral photographic product for providing diffusion transfer image patterns comprising:
  - a. an intensifier-emulsion layer which contains a particulate luminophor and a photosensitive silver halide system, the amount of particulate luminophor being sufficient to render said intensifier-emulsion layer substantially opaque and
  - b. a receiving layer arranged to receive a diffusion transfer image pattern from said intensifier emulsion layer.
2. A product of claim 1 wherein the ratio of particulate luminophor to silver is from about 7:1 to about 20:1.
3. A product of claim 1 further including a reflecting layer superposed on a support transparent to radioactive radiation and arranged so that said reflecting layer is interposed between said intensifier-emulsion layer and said support.
4. A product of claim 1 further including means for preventing visible light from striking the intensifier-emulsion layer.
5. A product of claim 4 wherein the means for preventing said visible light comprises a black dye which is alkali permeable and opaque to visible light but transparent to radioactive radiation and wherein the dye is coated on said intensifier emulsion layer.
6. A product of claim 1 further including an integral rupturable container confining an aqueous alkaline processing composition and wherein the container is integrated with the product so that upon rupture, the processing composition can be distributed between the intensifier-emulsion layer and the receiving layer.
7. A product of claim 1 wherein the particulate luminophor comprises zinc sulfide.
8. An integral photographic product which comprises:
  - a. a first support transparent to radioactive radiation and having thereupon a reflecting layer; and an intensifier-emulsion layer superposed on the reflecting layer, said intensifier emulsion layer comprising a particulate luminophor and a photosensitive silver halide system and wherein the amount of luminophor is sufficient to render the intensifier-emulsion layer substantially opaque;
  - b. a second support carrying a receiving layer arranged with respect to the intensifier-emulsion

11

- layer to receive a diffusion transfer image pattern therefrom and
- c. a rupturable container confining an aqueous alkaline processing composition and wherein the container is integrated with the product so that upon rupture, the processing composition can be distributed between the intensifier-layer and the receiving layer.

12

9. A product of claim 8 wherein the ratio of particulate luminophor to silver is from about 7:1 to about 20:1.

10. A product of claim 8 wherein the particulate luminophor comprises zinc sulfite.

11. A product of claim 8 wherein said first support comprises a base material opaque to visible light.

\* \* \* \* \*

10

15

20

25

30

35

40

45

50

55

60

65